

1

3,203,790

**EXTRUDED FLINTS AND PROCESS FOR  
MAKING SAME**

Walter Bungardt, Essen-Bredeney, Germany, assignor, by  
mesne assignments, to Ronson Corporation, Wood-  
bridge, N.J., a corporation of New Jersey

No Drawing. Filed Mar. 28, 1962, Ser. No. 183,023  
Claims priority, application Germany, Nov. 22, 1955,

G 18,429

12 Claims. (Cl. 75—152)

This is a continuation-in-part of application Serial No.  
623,798, filed November 23, 1956, now abandoned.

My invention generally relates to pyrophoric alloys  
and is more particularly directed to novel pyrophoric alloy  
compositions suitable for extrusion.

Considered from another aspect, my invention is con-  
cerned with an improved and simplified process for the  
extrusion of flints from pyrophoric alloy compositions and  
with the flints obtained thereby.

While flints for use in cigarette lighters and the like  
were originally produced by casting methods, such flints  
have, in recent years, been manufactured by extrusion,  
as extrusion, of course, increases the plant output, sim-  
plifies the manufacture and may be carried out with con-  
siderably less expenditure than casting methods. Fur-  
ther, the general quality of extruded flints including the  
pyrophoric characteristics compare favorably with and  
are in many respects superior to that of cast flints. For  
these reasons, the industry has generally adapted extru-  
sion processes for the production of flints.

Extruded as well as cast flints consist essentially of  
cerium (misch metal) iron alloys. However, those skilled  
in the art will readily realize that an alloy which may pro-  
duce satisfactory flints by casting is not necessarily suit-  
able as a raw material for extruded flints. This is so be-  
cause the problems and considerations underlying the ex-  
trusion of flints are entirely different from those prevail-  
ing in casting methods. In fact for many decades it  
was believed that the extrusion of cerium (misch metal)  
iron alloys was not feasible and in this connection I refer  
to my U.S. Patent 2,660,301 wherein I disclosed for the  
first time a commercially practical extrusion process for  
flint material and explained the obstacles which have to  
be overcome.

However, although my basic invention as embodied in  
said U.S. patent has been considered and proved to be a  
revolutionary advance in this particular art, the extrusion  
of flints from cerium (misch metal) iron alloys is still  
plagued by some serious problems. The most serious  
difficulty in the manufacture of flints or flint rods by ex-  
trusion from pyrophoric cerium (misch metal) iron alloys  
resides in the extremely high extrusion pressure which in  
present day processes is necessary for extruding the alloy  
composition through the extrusion die. Pyrophoric alloys  
used for the extrusion of flints ordinarily contain about  
4.5 to 40% of iron in addition to the cerium (misch metal)  
and such alloy composition can only be extruded at pres-  
sures between 5,000 to 16,000 kg. per square centimeter  
and at extrusion temperatures between 400-500° C. The  
particular pressure required is a function of the iron  
content in the alloy and increases with increasing amounts  
of iron. It is obvious that such high pressures require  
elaborate and excessively expensive extrusion presses,  
which moreover are, of course, subjected to considerable  
wear and tear. As the extrusion tools have to be fre-  
quently replaced and/or repaired, the intended gain and  
advantage by using extrusion instead of casting methods  
is therefore considerably negated or offset by the expen-  
diture in apparatus. In this connection, I wish to state  
that attempts have previously been made to reduce the  
extrusion pressure by alloying the basic alloy composi-

2

tion with additional metals. Thus in my own U.S. Patent  
2,792,301 I have disclosed certain metals which under  
stated conditions facilitate the extrusion.

In the production of flints by casting as distinguished  
from extrusion it has been suggested to add appreciable  
amounts of copper or zinc to the alloy mixture to increase  
the resistance of the flints to disintegration. Thus, U.S.  
Patents 2,408,400 and 2,389,198, for example, which are  
concerned with the production of flints by casting, recom-  
mend that at least 1.2% of copper are added in addition  
to silver, nickel and chromium. I have carried out ex-  
tensive experiments with this and other alloy composi-  
tions intended for casting with a view of ascertaining  
whether or not the teachings relating to the casting of  
flints could be beneficially made use of for the purpose of  
reducing the working pressure in the extrusion of flints.  
The results of my experiments are that these prior art  
casting compositions containing copper, zinc and other  
metals cannot in fact be extruded and therefore do not  
contribute anything of value to the extrusion art and par-  
ticularly have no bearing on the reduction of the extru-  
sion pressure. For the purpose of substantiating this con-  
tent, the following should be considered: The extru-  
sion of pyrophoric alloy compositions is by necessity car-  
ried out at temperatures at which the billet or ingot to be  
extruded is in a plastic state. If the optimum extrusion  
temperature is above the melting point of one or several  
of the metals of the alloy composition, this metal or  
metals liquify and the liquid phase seriously impairs the  
extrusion proper and in many cases renders extrusion im-  
possible. Thus, for example, I have attempted to extrude  
the alloy compositions disclosed in U.S. Patent 2,408,400  
and 2,389,198 previously referred to, but was not success-  
ful although I increased the extrusion pressure to 35 tons.  
The reason for my failure was that the composition  
formed a substantial amount of liquid phase which soiled  
and blocked the extrusion tools of the press.

It is, accordingly, a primary object of this invention to  
provide for an alloy composition which may be extruded  
at considerably lower pressures than was hitherto possible.

It is also an object of this invention to provide an ex-  
trusion process for the extrusion of flint material which  
may be carried out at lower pressure values than hereto-  
fore.

Another object of the invention is to provide extruded  
flints of excellent quality having superior pyrophoric  
characteristics.

Generally, it is an object of this invention to improve  
on the art of extruding flints as hitherto practiced.

Briefly, and in accordance with this invention, I have  
ascertained that the addition of small amounts of copper  
within predetermined limit ranges, to prior art extrusion  
alloy compositions considerably facilitates the extrusion  
procedure and permits the extrusion to be carried out at  
considerably lower pressure values than was hitherto  
feasible.

In my previous U.S. Patent 2,792,301, I have already  
suggested certain measures with a view to decreasing the  
required pressure for the extrusion procedure. Thus, in  
the prior patent referred to, I have proposed to admix  
the basic alloy composition with metals such as titanium,  
cadmium, magnesium, calcium, aluminum, barium, zir-  
conium or beryllium in predetermined quantities, i.e.,  
0.3% to 10%, preferably 0.3% to 1%.

I have found that although the admixture of the ele-  
ments referred to has in many instances a most beneficial  
influence on the reduction of the extrusion pressure, the  
addition of such metals within the stated ranges may some-  
times lead to difficulties and is therefore undesired. This  
is so because some of the enumerated metals, e.g. titanium  
and zirconium, alloy with the basic cerium (misch  
metal)-iron composition only with difficulty, particularly

if amounts in excess of 0.3% are employed. If the period for alloying the addition metals with the basic composition is protracted, the composition has to be maintained in molten condition for relatively long periods which, of course, results in metal losses. Further, some of the addition metals may adversely effect the corrosion resistance, shelf life and/or the pyrophoricity of the extruded flints.

In accordance with my present invention, I have conclusively established that small copper additions to the basic cerium (misch metal)-iron alloy composition overcome the drawbacks referred to and yet significantly reduce the extrusion pressure, provided the copper is added within a range of 0.05-0.45%.

The following Table I clearly establishes the beneficial effect on the working pressure of the addition of copper within the stated range.

TABLE I

| Test No. | Composition of alloy in percent by weight |      |      | Extrusion pressure in kg./cm. <sup>2</sup> at 480° C. and after 30 minutes of preheating treatment |
|----------|-------------------------------------------|------|------|----------------------------------------------------------------------------------------------------|
|          | Cerium (misch metal)                      | Fe   | Cu   |                                                                                                    |
| 468a     | 80.6                                      | 19.4 | 0.14 | 5,100                                                                                              |
| 469      | 80.46                                     | 19.4 | 0.24 | 3,500                                                                                              |
| 470      | 80.36                                     | 19.4 | 0.31 | 2,450                                                                                              |
| 471      | 80.29                                     | 19.4 | 0.45 | 2,250                                                                                              |
| 471a     | 80.25                                     | 19.3 | 0.55 | 2,100                                                                                              |
| 471b     | 80.15                                     | 19.3 | 0.55 | (*)                                                                                                |

\*Not extrudable because of partial liquefaction.

It will be noted that the extrusion pressure is 5100 kg./cm.<sup>2</sup> if the basic alloy composition is lacking copper, while copper additions to up to 0.45% result in a significant pressure reduction.

Further, it should be emphasized that the upper limit of 0.45% of copper is critical as larger amounts of copper in alloy compositions cause a partial liquification of the basic alloy composition. This is indicated in the table by test 471b. In this connection I refer to my above remarks and also to German Patent 891,824, where this matter has been dealt with in detail.

In analyzing the results of my tests as tabulated in Table I and considering the partial liquefaction of the alloy upon admixtures of copper in excess of 0.45%, I attempted to increase the copper content of the alloy while at the same time decreasing the extrusion temperature. As the partial liquefaction is, of course, dependent on the temperature, my reasoning was that a lowering of the working temperature would allow me to add larger amounts of copper without resulting liquefaction. The results of my tests in this regard were, however, very discouraging. While I succeeded in extruding alloy compositions containing up to 0.90% of copper at a temperature of 440° C., i.e. a temperature which is 40° C. lower than that of Table I, the extrusion pressure again rose to a considerable extent. My tests in this respect are tabulated in Table II.

TABLE II

| Test No. | Composition of alloy in percent by weight |      |      | Temperature and preheating | Extrusion pressure (kg./cm. <sup>2</sup> ) |
|----------|-------------------------------------------|------|------|----------------------------|--------------------------------------------|
|          | Cerium (misch metal)                      | Fe   | Cu   |                            |                                            |
| 471c     | 80.15                                     | 19.3 | 0.55 | 440°/15 min.               | 4,550                                      |
| 471d     | 79.7                                      | 19.4 | 0.90 | 440°/15 min.               | 4,300                                      |
| 471e     | 79.5                                      | 19.5 | 1.00 | 440°/15 min.               | (*)                                        |

\*Not extrudable because of partial liquefaction.

In comparing the results of Tables I and II it will be observed that, for example, a copper content of 0.90% requires an extrusion pressure of 4300 kg./cm.<sup>2</sup> at 440°

C., while the corresponding pressure is only 2100 kg./cm.<sup>2</sup> at 480° C. if the copper content is 0.45%. Therefore, the upper copper limit of 0.45% is critical if the extrusion pressure is to be reduced. In this connection it will be realized that from a practical point of view the reduction of the pressure is more desirable and important than a reduction in the working temperature.

According to another embodiment of my invention, I have ascertained that a further addition of one or several of the metals titanium, magnesium, calcium, beryllium, barium, aluminum and zirconium is effective further to reduce the extrusion pressure and to improve the quality of the extruded flints, provided these metals are added in minute quantities not exceeding 0.3%. Thus, if, for example, the basic cerium (misch metal)-iron composition is alloyed with 0.05-0.45% of copper and 0.2% of titanium or zirconium, the extrusion pressure is still further reduced.

Tests in this respect are tabulated in Table III.

20

TABLE III

| Test No. | Composition of alloy in percent by weight |      |      |                     | Extrusion pressure in kg./cm. <sup>2</sup> at 480° C. and after 30 minutes of preheating treatment |
|----------|-------------------------------------------|------|------|---------------------|----------------------------------------------------------------------------------------------------|
|          | Cerium (misch metal)                      | Fe   | Cu   | Additional elements |                                                                                                    |
| 528      | 80.2                                      | 19.6 | 0.21 | 0.20% Mg            | 4,800                                                                                              |
| 529      | 80.05                                     | 19.5 | 0.21 | 0.24% Mg            | 3,000                                                                                              |
| 530      | 79.95                                     | 19.8 | 0.25 | 0.25% Al            | 4,900                                                                                              |
| 531      | 79.92                                     | 19.6 | 0.25 | 0.23% Al            | 2,900                                                                                              |

The invention will now be described in connection with a specific example, it being understood, however, that this example is given by way of illustration and not by way of limitation, and that many changes may be performed without departing in any way from the scope and spirit of this invention as recited in the appended claims.

#### Example 1

This example illustrates test 471a of Table I above.

An alloy composition comprising 80.25% by weight of cerium (misch metal) and 19.3% of iron was alloyed with 0.45% of copper and cast into billet or ingot form. The alloy billet was thereafter heated to about 480° C. for 30 minutes and the billet was inserted into an extrusion press and was extruded into thin rods of 2 to 6 mm. diameter at an extrusion pressure of 2100 kg. per square centimeter. The extruded rods were thereafter cut down into individual flints of suitable length.

As control, the test was repeated with an alloy ingot which did not contain the copper addition. Extrusion only took place at a working pressure of at least 5100 kg. per square centimeter at the same temperature (see test 468a).

Similar tests were carried out to arrive at test results 469, 470, 471 and 471b.

While a specific embodiment of the invention has been shown and described in detail to illustrate the application of the inventive principles, it will be understood that the invention may be embodied otherwise without departing from such principles.

What I claim is:

1. A pyrophoric alloy composition suitable for extrusion essentially consisting of about 4.5 to 40% of iron and 0.05 to 0.45% of copper, the remainder being cerium (misch metal).
2. An extruded flint essentially consisting of about 4.5 to 40% of iron and about 0.05 to 0.45% of copper, the remainder being cerium (misch metal).
3. An extruded flint essentially consisting of about 18 to 22% of iron and about 0.05 to 0.45% of copper, the remainder being cerium (misch metal).
4. A pyrophoric alloy composition suitable for extrusion essentially consisting of about 4.5 to 40% of iron,

0.05 to 0.45% of copper, and a minute quantity of at least one metal selected from the group consisting of titanium, magnesium, calcium, beryllium, barium, aluminum and zirconium, said quantity being less than 0.3%, the remainder being cerium (misch metal).

5. An extruded flint essentially consisting of about 4.5 to 40% of iron, 0.05 to 0.45% of copper, and a minute quantity of at least one metal selected from the group consisting of titanium, magnesium, calcium, beryllium, barium, aluminum and zirconium, said quantity being less than 0.3%, the remainder being cerium (misch metal).

6. An extruded flint essentially consisting of about 18 to 22% of iron, 0.05 to 0.45% of copper and a minute quantity of at least one metal selected from the group consisting of titanium, magnesium, calcium, beryllium, barium, aluminum and zirconium, said quantity being less than 0.3%, the remainder being cerium (misch metal).

7. A process of producing flint rods by extrusion which comprises extruding a pyrophoric alloy in ingot form and essentially consisting of about 4.5 to 40% of iron and 0.05 to 0.45% of copper, the balance being cerium (misch metal) at a temperature of about 400 to 500° C. and at the lowest working pressure at which extrusion is possible.

8. The process as claimed in claim 7, wherein the alloy is preheated before being extruded.

9. The process as claimed in claim 7, wherein the extrusion pressure is about 2100 and 3500 kg./cm.<sup>2</sup>

10. A process as in claim 7, wherein the alloy addi-

20  
25  
30

tionally contains a minute quantity of at least one metal selected from the group consisting of titanium, magnesium, calcium, beryllium, barium, aluminum and zirconium, said quantity being less than 0.3%, the remainder being cerium (misch metal).

5. 11. In a process of extruding flints from alloy compositions in ingot form, wherein the alloy composition essentially consists of about 4.5 to 40% of iron, the remainder being cerium (misch metal), and the alloy composition is extruded at a temperature of about 400-500° C., the improvement which comprises incorporating into the alloy composition, prior to extrusion, 0.05 to 0.45% of copper to reduce the required extrusion pressure.

12. A process as in claim 11, wherein the alloy composition additionally contains a minute quantity of at least one metal selected from the group consisting of titanium, magnesium, calcium, beryllium, barium, aluminum and zirconium, said quantity being less than 0.3%, the remainder being cerium (misch metal).

#### References Cited by the Examiner

##### UNITED STATES PATENTS

|           |       |          |          |
|-----------|-------|----------|----------|
| 2,408,400 | 10/46 | Kent     | 75-152   |
| 2,792,301 | 5/57  | Bungardt | 75-135 X |

##### FOREIGN PATENTS

|           |       |          |
|-----------|-------|----------|
| 1,017,507 | 10/57 | Germany. |
|-----------|-------|----------|

DAVID L. RECK, Primary Examiner.

30